

## 1

3,172,763

**STRONTIUM CHROMATE LIGHT-SENSITIVE  
CARBON TISSUE**

Charles A. Kumins, Chappaqua, and Daniel Smith, Riverdale, N.Y., and Rudolf G. Frieser, Neshanic Station, N.J., assignors to Interchemical Corporation, New York, N.Y., a corporation of Ohio  
No Drawing. Filed May 12, 1961, Ser. No. 109,511  
4 Claims. (Cl. 96—75)

This invention relates to the manufacture of so-called "carbon tissues" employed in the photomechanical reproduction art. These tissues are employed in preparing etched printing plates or rolls from copy which may be a photographic transparency of a line drawing or of a many-toned subject. They are also of use in preparation of gelatin reliefs for use in printing by the imbibition processes. This application is a continuation-in-part of our application Serial No. 683,969, filed September 16, 1957.

Up to the time of our present invention, it has been the practice to use carbon tissues consisting essentially of light sensitive coated papers, such as light sensitive gelatin coated papers. The sensitized coating may contain minor amounts of other ingredients, such as pigment (to make the relief image more readily visible and to control penetration of actinic radiation into the gelatin layer) and such materials as soaps, sugar, glycerin, etc., to improve its physical properties. Because lamp-black was formerly used as the pigment in coating such papers, they came to be known as "carbon tissues"; other pigments are now commonly employed, among them finely powdered iron oxide, such as jewelers' rouge.

Carbon tissues as presently manufactured are quite stable in storage and essentially insensitive to light. Before use, however, it is necessary to sensitize them by wetting them thoroughly with a sensitizing solution of a salt of hexavalent chromium, usually a dilute solution of an alkali dichromate, such as ammonium dichromate, sodium dichromate, or potassium dichromate. After being thoroughly wetted with sensitizing solution, the tissue must be dried and used rather promptly. The sensitivity of the dried tissue changes with storage, and tissue at least one day old is preferred for carbon printing because the initial changes in sensitivity are so rapid and large as to produce results variable beyond the limits of commercial tolerance. Storage for more than a week after sensitization is impractical since, even without exposure to light, the gelatin hardens gradually, and can then no longer be differentially insolubilized by exposure to light and then partially dissolved to form a satisfactory relief image.

The mode of employment of "carbon tissues" is familiar to those well-versed in the printing and photographic arts, and, since it constitutes no part of our invention, will not be further described here, except insofar as necessary to describe our invention.

It is an object of our invention to provide a new type of coating whereby storage-stable, light-sensitive carbon tissues may be prepared. A further object is to provide a process of producing an emulsion of extremely finely divided water-insoluble chromate pigments.

It is a still further object of our invention to provide a carbon tissue which is sensitized at the time of manufacture and which is stable enough in storage as to permit

## 2

it to be stocked ready for use by jobbers and the ultimate user. It is another object to provide a method of producing such a carbon tissue. Other objects will become apparent from the detailed description of our invention which follows.

Surprisingly, we have found that if we coat paper or other flexible water-insoluble membrane with an aqueous solution of gelatin, or an equivalent sensitizable material, containing dispersed therethrough extremely small and uniform-sized particles of a substantially water-insoluble chromate, preferably strontium chromate, a tissue is obtained which has all the desirable properties of carbon tissue freshly sensitized by the previously known method and which, in addition is capable of being stored before use for periods up to six months or even a year. The advantages of such a product are obvious, and the industry has long sought in vain for such a material.

While we do not wish to be bound by or limited to any theory or attempted explanation as to the reactions involved in the practice of our invention, we believe, on the basis of our study and experiments, that the effect of light on the chromated gelatin is to convert chromate (or bichromate) ion to chromic ion, and that the chromic ion so formed acts to denature (i.e., harden or insolubilize) the gelatin. These reactions appear to occur slowly even without the influence of light when the chromate or bichromate ions are in solution, so that after brief storage the gelatin of a conventional carbon tissue sensitized in the usual manner becomes hardened throughout and is no longer usable for the preparation of a gelatin relief image. We have found that this rapid deterioration of the sensitive material does not occur when the chromate is present as a water-insoluble solid.

In order to prepare satisfactory carbon tissues according to our invention, it is important that the insoluble chromate dispersed in the gelatin be in an extremely fine state of subdivision. This aids in the uniform distribution throughout the gelatin necessary for uniformity of the coating, increases transparency, and makes for greater photosensitivity.

We have found that desirably fine-particle chromates can be prepared by precipitation in an aqueous system of increased viscosity. Preferably for the purpose of preparing coatings for our novel carbon tissues, we employ gelatin for increasing the viscosity of the reaction medium, though other thickening agents, including gum arabic, gum tragacanth, and other natural and synthetic thickening agents may be employed.

We have found it possible to employ the chromates of several different metals in the practice of our invention, including lead, silver, strontium, and barium. We have found strontium chromate to give tissues of excellent sensitivity, shelf life, and scale-gradation, and accordingly prefer it for use in our invention. For precipitating the insoluble chromates for use in coating our novel carbon tissues, any soluble salt of strontium, lead, silver, or barium may be used in the practice of our invention, but for reasons of economy, availability, and convenience, we prefer the nitrates. Similarly, the choice of a soluble salt of hexavalent chromium employed is not particularly critical. For economy and convenience we prefer sodium dichromate, though ammonium dichromate is equally suitable.

The particle size of the insoluble chromates dispersed in gelatin according to our novel process is very uniform

and is generally about 100-1000 Angstrom units. The particles appear to be spheres, and so differ from the much larger rod-shaped particles in which lead and strontium chromates are obtained by ordinary precipitation methods.

The following examples illustrate our invention.

*Example I*

Fifty parts of unflavored edible gelatin (Knox's) and 10 parts of jewelers' rouge are added to 250 parts of warm (60° C.) water, and stirred until a homogeneous mixture is obtained. This mixture is allowed to cool to 40° C. (while stirring is continued), and 19.1 parts of anhydrous strontium nitrate is added. After the strontium nitrate is dissolved, a solution of 13.4 parts of sodium dichromate dihydrate in 250 parts of water is added slowly over a period of about an hour. The mixture is then brought to a pH of between 7 and 8 by the addition of about 10 parts of concentrated ammonium hydroxide solution. Stirring is continued for 20 minutes, after which the emulsion is bottled, cooled to room temperature, and stored in the dark. From the time of commencing the addition of dichromate to the time of bottling, the temperature of the mixture is maintained at about 40° C. and all operations are carried out in the dark or in weak, diffused, preferably yellow, light. The emulsion may be used at once for coating paper, or may be stored for several days. It is inadvisable to store the wet emulsion for a very long time, however, since it deteriorates on standing, and may become entirely inactive if stored for a month at room temperature.

A bottle containing the emulsion prepared above is placed in a warm water bath to heat its contents to about 40° C. and convert the gel to a flowable liquid. This liquid is flowed onto a smooth-surfaced paper to produce a uniform coating. The paper is then transferred promptly to a cold environment to cause setting of the gelatin. (A household-type of refrigerator provides satisfactory cooling for small lots of tissue.) After setting of the gel, the tissues are dried in a current of air. Prompt cooling of the coated tissue is desirable so as to avoid penetration of the paper, as this would interfere with later stripping. The speed of drying is somewhat less critical, but since the undried coating emulsion has only limited storage stability, it is preferably to reduce the water content rather promptly to assure uniformly sensitive tissues of good stability in storage. All operations in the preparation of the carbon tissue are conducted in weak, preferably yellow, light, but there is no need for total darkness; the working space may be comfortably lighted, so long as direct sunlight or intense artificial light is avoided.

The tissue prepared above may be employed in the well-known manner for the preparation of gelatin washoff relief images for imbibition printing or resists for etching of printing plates or rolls. Exposure may be by sunlight, carbon, mercury vapor, or rare gas arcs, or by tungsten filament lamps.

The exposed tissues may be transferred in the usual manner to polished metal, paper, Celluloids, or the like. The relief images may be developed in the usual manner with warm water. Metal plates or rolls on which the relief images are developed may be etched with the usual etching solutions, such as aqueous ferric chloride.

*Example II*

Nineteen grams of strontium nitrate are dissolved in a solution of 200 grams of gum arabic in 250 milliliters of water at 40° C. A solution of 13.4 grams of sodium dichromate dihydrate in 250 milliliters of water is added dropwise to the strontium nitrate solution and then 10 milliliters of ammonium hydroxide (28%) is added. Stirring is continued for 20 minutes, after which the emulsion is bottled, cooled to room temperature, and stored in the dark. From the time of commencing the addition of dichromate to the time of bottling, the temperature of

the mixture is maintained at about 40° C., and all operations are carried out in the dark or in weak, diffused, preferably yellow, light.

To prepare carbon tissue from the above emulsion, it is 5 coated on a smooth-surfaced paper to produce a uniform coating of approximately 0.3 mil thickness using a Mayer hand coating apparatus. The coated tissues are dried in a current of air. All operations in the preparation of the 10 carbon tissue are conducted in weak, preferably yellow light. The tissue is used in a manner similar to that of the tissue of Example 1.

*Example III*

Using a procedure similar to that of Example II a chromated emulsion was prepared from

- (A) 250 grams of a 7.5% aqueous solution of carboxy methyl cellulose gum (Hercules CMC, Type 7MS) described by the supplier as a moderately low molecular weight material having a viscosity of 2 to 8 poises (2% solution in water at 25° C.) with approximately 25% of the available groupings in the original cellulose substituted by carboxy methyl groups,
- (B) 10 grams of strontium nitrate,
- (C) 13.4 grams of sodium dichromate dihydrate in 250 milliliters of water, and
- (D) 10 milliliters of ammonium hydroxide (28%).

A carbon tissue was prepared according to the procedure in Example II and exposed to a carbon arc source through 30 a conventional high contrast line negative. Five seconds exposure gave a well defined image, with the unexposed portions being readily removable by washing at 120° F.

*Example IV*

In a manner similar to that of Example II a light sensitive emulsion was prepared from

- (A) 150 grams of Elvanol 51-05 dissolved in 250 milliliters of water. (Elvanol 51-05 is described by the supplier as a low molecular weight polyvinyl alcohol having a viscosity of 4.2 centipoises as measured in a 4% aqueous solution at 20° C., a pH of 5.9, and an 88.2% hydrolyzed polyvinyl acetate.)
- (B) 19 grams of strontium nitrate,
- (C) 13.4 grams of sodium dichromate dihydrate in 250 milliliters of water,
- (D) 10 milliliters of ammonium hydroxide (28%).

This emulsion gave a light sensitive coating on paper of less sensitivity than the emulsion of Example III in that it required about 30 seconds' exposure to develop an image as against five seconds for the coating of Example III.

From the above examples it is evident that the above invention has general applicability to the preparation of light sensitized coatings in general.

We claim:

1. A light-sensitive relatively storage stable carbon tissue comprising a flexible, water-insoluble, supporting membrane, coated with a thin, substantially uniform light-sensitive emulsion layer comprised of a material of the group consisting of gelatin, polyvinyl alcohol, carboxy methyl cellulose and gum arabic in which is dispersed a finely divided strontium chromate as a photosensitizing component.
2. A product according to claim 1 in which the average size of the strontium chromate particles is less than 1000 Angstrom units.
3. A light-sensitive relatively storage-stable carbon tissue comprising a flexible, water-insoluble supporting membrane coated with a thin, substantially uniform layer of gelatin in which is dispersed a finely divided strontium chromate as a photosensitizing component.
4. A product according to claim 3 in which the average size of the strontium chromate particles is less than 1000 Angstrom units.

## References Cited in the file of this patent

## UNITED STATES PATENTS

|           |               |               |
|-----------|---------------|---------------|
| 428,472   | Dubois -----  | Mar. 16, 1887 |
| 1,984,090 | Seymour ----- | Dec. 11, 1934 |
| 2,162,618 | Izard -----   | June 13, 1939 |
| 2,902,390 | Bell -----    | Sept. 1, 1958 |

## FOREIGN PATENTS

|                  |                     |               |
|------------------|---------------------|---------------|
| 97,115           | Germany -----       | Mar. 21, 1898 |
| 1,983<br>of 1856 | Great Britain ----- | Aug. 26, 1898 |
| 435,337          | Canada -----        | June 18, 1946 |

## OTHER REFERENCES

Canadian Patent Office Record, vol. 74, 1946, page 1479.

<sup>5</sup> Handbook of Chemistry and Physics, Chemical Rubber Publishing Co., Cleveland, Ohio, 35th edition, 1953-1954, pages 604-605.

Kuhne, Farbe and Lack: Centralblatt, 1930, pages 243-244, 23-56.

<sup>10</sup> Tritton: The Photographic Journal, pages 281-285, June 1929.

Kolthoff et al.: Volumetric Analysis, vol. 3, page 335. Interscience Publishers Inc., N. Y., 1957.